

Jan. 13, 1925.

A. L. D. D'ADRIAN

1,523,103

METHOD OF OBTAINING METALS FROM THEIR RESPECTIVE OXIDES OR ORES

Filed March 12, 1920



INVENTOR  
*Alexander L. Duval D'Adrian,*

BY  
*C. P. Goepel*  
ATTORNEY

Patented Jan. 13, 1925.

1,523,103

# UNITED STATES PATENT OFFICE.

ALEXANDER L. DUVAL D'ADRIAN, OF WASHINGTON, PENNSYLVANIA.

## METHOD OF OBTAINING METALS FROM THEIR RESPECTIVE OXIDES OR ORES.

Application filed March 12, 1920. Serial No. 365,181.

To all whom it may concern:

Be it known that I, ALEXANDER L. DUVAL D'ADRIAN, a citizen of the Republic of France, and a resident of Washington, 5 county of Washington, and State of Pennsylvania, have invented certain new and useful Improvements in Methods of Obtaining Metals from Their Respective Oxides or Ores, of which the following is a 10 specification.

In the reduction of certain metals from their respective oxides in the presence of carbon by an electric arc, disadvantages have appeared in the considerable expense 15 involved in the replacement of the carbon or graphite electrodes, and further disadvantages have appeared in the fact that the carbon with which the oxides are mixed, is not altogether eliminated, but to some 20 extent combines with the reduced metal.

One of the objects of my invention is to overcome these undesirable features, and to provide a novel method in the use of which a metal is obtained which is practically pure and free from carbon or carbon combinations, and which novel method is attendant with a lower cost of operation than those hitherto employed.

To enable my improved method to be 30 understood, I will now describe the same by referring to one embodiment of my invention. I take the quantity which is desired to be treated, of a metallic oxide, and grind it to a fine powder. In order to get 35 a thorough mixture with carbon, I mix this ground oxide with carbon of the proper amount, and then thoroughly grind the mixture, this amount of carbon depending to some extent on the character of the 40 oxide, as outlined in the following table of typical metallic oxides:

| 45 | Oxide.                                                 | Atomic weight element. | Molecular weight of oxid. | Theoretical amount of carbon required for one pound of oxide. | Pounds. |
|----|--------------------------------------------------------|------------------------|---------------------------|---------------------------------------------------------------|---------|
| 50 | Barium BaO.....                                        | 137.37=                | 153.37                    | 0.0391                                                        |         |
|    | Cobalt CoO.....                                        | 58.98=                 | 74.97                     | 0.1017                                                        |         |
|    | Tungsten WO <sub>3</sub> .....                         | 184. =                 | 232.0                     | 0.0776                                                        |         |
|    | Vanadium V <sub>2</sub> O <sub>3</sub> .....           | 51.0 =                 | 150.0                     | 0.12                                                          |         |
|    | Uranium U <sub>3</sub> O <sub>8</sub> .....            | 238.2 =                | 842.6                     | 0.0569                                                        |         |
|    | Chromium Cr <sub>2</sub> O <sub>3</sub> .....          | 52.0 =                 | 162.00                    | 0.1184                                                        |         |
|    | Molybdenum sesqui Mo <sub>2</sub> O <sub>5</sub> ..... | 96.0 =                 | 240.00                    | 0.075                                                         |         |
|    | Molybdenum tri-oxide MoO <sub>3</sub> .....            | 96.0 =                 | 144.00                    | 0.125                                                         |         |
| 55 | Molybdenum di-oxide MoO <sub>2</sub> .....             | 96.0 =                 | 128.00                    | 0.0937                                                        |         |
|    | Uranium dioxide UO <sub>2</sub> .....                  | 238.2 =                | 270.20                    | 0.0444                                                        |         |

varying with the character of the metal. I prefer a mixture of both fluor spar and lime with silica. I prefer to arrange the electrodes in a furnace provided with an arc, as shown in the annexed drawing: In this drawing 5 designates the furnace structure of a suitable refractory material, which is arranged upon a foundation or support 6. The furnace chamber 7, in which the molten metal is collected, is provided with an outlet passage 8 extending through one side of the furnace structure and directing the molten metal into a trough or spout 9 projecting laterally from the furnace.

10 indicates a curved refractory arched wall extending over the furnace chamber, and having openings 11, through which the electrodes formed in the manner above set forth protrude into the chamber 7. Preferably these electrodes extend in a convergent relation to each other so that their lower ends within the furnace chamber are spaced a suitable distance apart for the formation of the electric arc. The arch 10 is normally provided with a central opening 12 affording a free exit for the gas which is generated in the reduction of the metallic constituent of the electrodes to a molten condition.

The outlet end of the discharge passage 8 is normally closed by means of a suitable plug 14.

The intensity of the current depends upon the material to be treated, some oxides requiring only sixty volts, others eighteen hundred volts, and still others several thousand, depending upon the conductivity of the molded electrodes.

40 As a modified form of my method, I shape the electrodes with a finely ground core of coke or some other form of carbon (which, for instance, in the case of the reduction of cobalt oxides is not necessary), to increase the conductivity of the electrodes. In this case, the carbon of the mixture and the carbon of the core equal the necessary amount of carbon to reduce the oxide to metal.

50 By the methods described, metals may be obtained in practically pure state from their respective oxides, as for instance, cobalt, nickel, tungsten, uranium, chromium, molybdenum, zirconium, vanadium, tantalum, thorium, and in fact any metal which has sufficient value to make the use of the process sufficiently remunerative.

60 The above-described method is also adapted for the production of ferro-alloys. In this case, iron, preferably finely divided, can be added in suitable amounts to the mixture used to form the electrodes above described. On the other hand, when iron is also present in ore containing another metal 65 in the form of an oxide, as for example,

chromite used for obtaining ferro-chromium, additional chromium oxide may be added to the mixture, in case the proportion of iron in the ore exceeds that desired in the ferro-chromium or vice versa, iron may be added should the proportion of chromium oxide in the chromite be higher than that desired in the ferro-chromium. In other words, the mixture to be formed into electrodes is so proportioned that the desired ferro-alloy which is secured by the action of the arc between the electrodes, has the proportions desired.

I have disclosed a satisfactory manner of carrying out my improved method or process, but it will be understood that certain modifications may be made therein without departing from the spirit of my invention as defined in the appended claims.

What I claim as new and desire to secure by Letters Patent is:

1. The process of obtaining metals from their respective oxides, which consists in forming the oxide mixed with carbon into electrodes, and then establishing an electric arc between the ends of the electrodes, for producing an intensive heat, thereby reducing the oxides to metal without the substantial production of slag.

2. The process of obtaining metals from their respective oxides, which consists in grinding the carbon and oxide together, then molding with a binder the mixture in the form of electrodes, and then by means of an electric arc reducing the metal of the oxide without the substantial production of slag.

3. The process of obtaining metals from their respective oxides, which consists in molding a mixture of the metallic oxide to be reduced, carbon and a binder in the form of an electrode, then baking the same at about 1000° C. or over, without undue access of air, to accomplish a partial reduction of the oxide, and then establishing an electric arc between a pair of electrodes to complete the reduction of the oxide into metal.

4. The process of obtaining metals from their respective oxides, which consists in adding carbon and a binder to ground oxides, and molding the mixture around a central core of coke or other form of carbon into electrodes, and then establishing an electric arc between the electrodes so formed, to reduce the oxides to metal.

5. The method of obtaining a ferro-alloy which consists in mixing iron and a metallic oxide and carbon in proportions to correspond to the composition of the ferro-alloy desired to be produced, forming the mixture into electrodes, and producing by the action of the electric arc, a ferro-alloy.

6. The process of obtaining metals from ores comprising forming the ore and a re-

ducing agent into electrodes and recovering the metal-content thereof in a metallic condition by the application of heat without the substantial production of slag.

7. The process of obtaining metals from ores comprising forming the ore and a reducing agent into electrodes and recovering the metal-content thereof in a metallic condition without the substantial production of slag by establishing an electric arc between the electrodes.

8. The process of obtaining metals from compounds thereof comprising forming a mixture of the compound, a reducing agent and a binder in the form of an electrode, baking the same at about 1000° C. to accomplish a partial reduction of the metal compound and thereafter reducing the same by the application of electrically generated heat.

9. As a new article of manufacture, an electrode comprising the reaction-products formed by baking a mixture of a reducible compound, a reducing agent and a binder at a temperature of about 1000° C. 25

10. As a new article of manufacture, an electrode comprising the reaction-products formed by baking a mixture of a metallic oxide, a reducing agent and a binder at a temperature of about 1000° C. 30

11. As a new article of manufacture, an electrode comprising the reaction-products formed by baking a mixture of a reducible oxide, a reducing agent and a binder at a temperature of about 1000° C. 35

In testimony that I claim the foregoing as my invention, I have signed my name hereunder.

ALEXANDER L. DUVAL D'ADRIAN.